# EUROPEAN PATENT SPECIFICATION

(11) **EP 2 110 446 B1**
(45) Date of publication and mention of the grant of the patent: **19.02.2014**
(21) Application number: 08154833.1
(22) Date of filing: 18.04.2008
(51) Int. Cl.: C14C 3/10

(54) **Tanning of hides and skins**
Gerbung von Fellen und Häuten
Tannage de cuirs et de peaux

(43) Date of publication of application: 21.10.2009
(73) Proprietor: C & J CLARK INTERNATIONAL LIMITED, Street Somerset, BA 16 0EQ (GB)
(72) Inventor: Booth, Stuart, Northampton, Northamptonshire NN3 6JD (GB)
(74) Representative: Marles, Alan David

(56) References cited:
- DE-C- 905 054
- FR-A- 926 892
- DATABASE WPI Week 200275 Thomson Scientific, London, GB; AN 2002-693877 XP002496059 & JP 2002 180099 A (TEIKOKU KASEI KOGYO KK) 26 June 2002 (2002-06-26)

## Description

### Field of the Invention

The present invention relates to methods of tanning hides or skins.

### Background of the Invention

Tanning of hides or skins to produce leather is an ancient process that takes advantage of the property of hides or skins that they absorb tanning chemicals that prevent putrefaction, increase resistance to moisture and promote suppleness.

The tanning process involves the reaction of the tanning chemicals with collagen fibres present in the hide or skin. The most common tanning chemicals are chromium based compounds (e.g. chromium sulfate), synthetic tanning chemicals, alum, aldehydes (e.g. formaldehyde) and vegetable tanning compositions.

Vegetable tanning compositions are composed of polyphenolic compounds, with the tanning properties related to the size of the molecule and the number of phenolic -OH groups. Vegetable tanning compositions are sometimes referred to as "tannins". Although the term "tannin" refers to the ancient use of some tannins in the tanning process, the term is now widely applied to any plant-derived large polyphenolic compound containing sufficient hydroxyls and other suitable groups (e.g. carboxyl groups) to form strong complexes with macromolecules whether or not such compounds have previously been used to tan hides or skins.

Vegetable tannins used in tanning are derived from tree bark, in particular, the bark of oak, chestnut, quebracho and mimosa.

FR-A-926892 discloses the tanning of hides or skins with aqueous extracts of pulverised oil cake from residues of olive fruits.

DE-C-905054 discloses the use of myrobalane fruits in the tanning of leather.

JP 2002180099A discloses the tanning of hides or skins with tannin extracts from Tara fruit sheath.

There is a need for improved tanning processes that have a lesser environmental impact and yet still provide leather of good quality.

It is an object of the present invention to address this need.

### Summary of the Invention

The present invention accordingly provides, in a first aspect, a method of tanning hides or skins, the method comprising a fruit tanning step of contacting, for a predetermined time and at a predetermined temperature, a hide or skin with a tanning liquor comprising a fruit tanning extract, characterised in that the fruit tanning extract is derived from cider apples, and wherein the tanning liquor also comprises one or more vegetable or synthetic tanning agents, and in that the fruit tanning step is a fruit re-tannage step, the predetermined time is from 6 to 48 hours and the predetermined temperature is from 25°C to 85°C.

The advantage of using a fruit tanning extract is that it is possible to use fruits which are readily available and do not involve the felling, for example, of trees but are an annually renewable resource.

The fruit is an edible fruit. This is advantageous because edible fruits are produced in large quantities and a large amount of edible fruit waste is available.

The fruit will be a fleshy fruit.

The fruits are of the sub-family Maloideae (also known as Pomoideae).

Maloideae fruits are produced in large quantities throughout the world and typically contain relatively large quantities of polyphenolic compounds. The fruit is a pome, in particular, an apple. Apples are known to contain polyphenolic compounds, including quercetin, catechin, gallic acid, phloretin and chlorogenic acid. Surprisingly, it has been discovered that these compounds have properties that make them suitable for use in tanning of hides or skins. Apples are particularly advantageous because the apple, apple juice and cider industries (cider being an alcoholic beverage produced from apples) produce large quantities of apples and waste products, much of which will contain these polyphenolic compounds.

The content of polyphenolic compounds in apples depends very much on the variety of the apple, as well as climate and other growing conditions. Typically, apples grown under low nitrogen regimes or adverse weather conditions tend to contain more polyphenolic compounds. These compounds are also increased in amount if nutrients are restricted during the growing season of the apple. There is also a possibility of using unripe apples which typically contain higher quantities of the polyphenolic compounds.

The type of apple is a cider apple. The use of cider apples is advantageous because many cider apples contain high quantities of polyphenolic compounds and also because, typically, the flesh of the apple has a fibrous texture making it easier to extract the juice.

There are a large number of traditional cider apple varieties grown in, for example, England. Of these varieties, the preferred varieties for use in the method of the present invention are bittersweet and bittersharp cider apples. Bittersweet apples impart the characteristic flavour of English West Country ciders and are typically low in acid and high in polyphenolic compounds (the "tannin" component of the cider). Bittersharp apples are relatively high both in acid and polyphenolic compounds. Examples of varieties of bittersweet or bittersharp apples include Michelin or Dabinett.

Preferably, the method of the present invention further comprises one or more further tannage steps. These tannage steps may be vegetable or synthetic tannage steps and may take place either before or after the fruit tanning step.

The method may also further comprise one or more of the following steps after the fruit tanning step: neutralisation, fatliquoring, fixation and finishing. Similarly, the method may comprise one or more of the following steps before the fruit tanning step: soaking, liming and/or dehairing, fleshing, splitting, pickling, samming and shaving.

In a preferred embodiment of the present invention, the fruit tanning step is a fruit retannage step. In this embodiment, the fruit tanning step takes place after a first tannage step which, as discussed above, may involve a vegetable (e.g. chestnut, oak, mimosa or other tree bark or wood extract) or synthetic tanning agent.

There may be one or more tannage steps before the fruit retannage step.

The tanning liquor also comprises one or more vegetable or synthetic tanning agents in addition to the fruit tanning extract. Typically, the fruit tanning extract would be between 20 and 60% of the tanning liquor usually by weight, occasionally by volume. Preferably, the fruit tanning extract would be between 25 and 50%, more preferably between 25 and 40% of the tanning liquor. If dried fruit tanning extract were to be used then the dried (e.g. spray dried) fruit tanning extract would be between 5 and 25% preferably 5 and 20% and most preferably 5 and 15% of the tanning liquor by weight.

It is advantageous if the predetermined time involved in the fruit tanning step is from 6 hours to 48 hours, preferably from 6 to 36 and more preferably from 12 to 24 hours. The predetermined temperature is preferably from 25 to 85°C, more preferably from 25 to 50°C, most preferably from 25 to 40°C.

In the method according to the invention, the fruit tanning extract is preferably obtainable by aqueous extraction of pulped fruit at elevated temperature. Alternative extraction methods which may be used include solvent extraction or aqueous extraction by boiling under pressure.

The benefit of aqueous extraction at elevated temperature not under pressure is primarily one of cost but it also reduces the likelihood of degradation of the polyphenolic compound in the fruit extract.

The elevated temperature is preferably between 40 and 100°C, more preferably between 50 and 80°C and most preferably between 50 and 75°C.

The pulped fruit from which the fruit tanning extract is obtained in the most preferred embodiment is apple pomace either before or after pressing of the juice for cider. The apple pomace may be either wet pomace or dried pomace (e.g. spray dried pomace) or a mixture of the two.

### Detailed description of the invention

The invention will now be further illustrated by a detailed description of a method of tanning bovine hides using fruit tanning extracts derived from apples.

In cider production, apples are washed prior to milling (comminution) so that leaves, twigs, silt etc. are removed. The wet pomace waste after pressing is unstable and susceptible to microbiological attack, and so it is usually spray dried within minutes of pressing to prolong storage time. The waste requires dry storage in a darkened room/area to avoid oxidation by light.

Trials were carried out using simple aqueous extraction of wet or dry apple waste by heating in water at 70°C, aqueous extraction under pressure and solvent extraction. The tannin content was measured using the Official SLTC method and the Lowenthal Permanganate Titration method (as used in the cider industry). There is a difference in the tannin content between the wet and dry apple wastes. The results showed that for the dry apple waste (using the Lowenthal Permanganate Titration) the tannin content is about 0.06% by weight compared to about 0.04% by weight for the wet apple waste.

There was no advantage in using the more expensive routes of extraction by aqueous boiling under pressure or solvent extraction (using e.g. toluene) so simple heated water extraction (70°C) was chosen. This aqueous system gives several environmental advantages including avoiding the need to remove the solvent by distillation and keeping the COD lower.

### Method for tannin extraction

The spray dried apple waste is weighed and introduced into a tanning processing drum. 700% of water (relative to the weight of apple waste) is added at 74°C and the drum is run to obtain a homogenous mix. After 5 min the temperature is checked and a further 120% of water at 80°C is added. At this stage the extract is a viscous slurry at temperature of 60°C. The process is run for a further 2.5 hours with continuous monitoring of temperature and appearance.

On completion of the extraction, 0.08% of biocide (Myacid AS) is added to reduce the potential for putrefaction. The process is run for a further 10 min and left overnight to cool.

The following day, the drum is run for 10 min to re-mix the extract which is then filtered using either an Archimedean screw technique or filter press. To avoid putrefaction, a further 0.04% of biocide and 0.04% of fungicide are added to the final extracted liquid. In total 80 kg of dried pomace results in about 220 kg of liquid tannin extract being obtained with a moisture content of 96% by weight and 4% unfiltered solids. Analysis (of the liquid phase) indicated a tannin content of 1-2 weight %.

### Tanning Process

The liquid tannin extract obtained from the apple extraction is used in combination with vegetable tannins and syntans to tan bovine hides to produce leather.

### 1. Preparation

The hides are prepared for tanning using the conventional beamhouse process of soaking, liming, fleshing, splitting, and pickling. They are then sammed and shaved to 1.1 - 1.2 mm substance and placed into a drum containing 150% water and 0.5% oxalic acid to minimise the iron staining. They are washed with water at 20°C and are ready for tanning.

### 2. Tannage

During the tanning process the collagen fibre is stabilized and converted to leather by the cross-linking action of the tanning agents rendering the hide no longer susceptible to putrefaction. Tanning also increases the tensile strength and heat resistance.

Following the washing process, the hides are pretanned using 70% water, 2% Paralene PGS and 2% Sellasol SL. These syntans assist penetration of the vegetable tanning chemicals. This is followed by the main vegetable tannins using 10% Quebracho ATO, 5% Mimosa and 5% Chestnut. This process lasts for 60 min at 20°C.

### 3. Apple re-tannage

Following this main tannage, the apple retanning is carried out in a separate process using 100% water, 45% liquid apple tanning extract, 5% Chestnut, 5% Fitapor GT, 1.5% of Manacryl SRG and 1% of Dermadol ID. Thus a blend of apple tannin and conventional vegetable retanning agents and a resin retannage are used. This process takes place at 30°C for 6 hours and is then run intermittently overnight (5min/hour). The retanning process improves the feel and handle of the leather, fills the looser parts of the leather, improves the resistance to alkali, perspiration and general wear characteristics.

### 4. Neutralisation

Following retannage, a light oxalic acid wash is given again to minimise the risk of iron staining, using 100% water at 30°C and 0.5% oxalic acid for 30 min. This is followed by neutralisation with 50% water at 40°C, 2% sodium formate and 4% Dermaflex FR/C to obtain pH 4.5-4.8. This assists penetration of the subsequent fatliquoring.

### 5. Fatliquoring

The fatliquoring is a combination of 8% Dermadol BK, 3.5% Dermadol MC, 1.5% Dermadol ID and 5% Tresin ML Liq for 60 min. Leathers are fatliquored to lubricate the fibres and achieve product-specific characteristics of softness and drape.

### 6. Fixation

At the end of the process, the leathers are given a last oxalic acid wash and a little syntan to dry the surface. The final treatment is fixation of the chemicals with 1% Remsol ALM and 1% formic acid.

The process of steps 1 to 6 is further described in Table 1.

### 7. Finishing

To enhance the appearance of the leather and provide the performance characteristics expected, finishing operations are carried out. A range of mechanical finishing operations such as buffing/dedusting, dry milling (mechanical softening) and polishing are carried out. A surface coat is also applied to provide protection, hand feel, colour and gloss and to meet the customer requirements.

### 8. Leather produced by the process

Leather produced by the method according to the invention is of excellent quality with very similar properties of suppleness and other properties to leather produced using a conventional process.

### Spray drying of liquid tanning extract

Trials were conducted using liquid tanning extract which had been spray dried. A sample of 5 kg of apple liquid tanning extract was spray dried producing approximately 50 g of spray dried extract. The spray dried extract may be used in the tanning process in place of the liquid tanning extract, with important advantages in reducing dilution and hence allowing an increased fruit tannin content in the tanning process.

**Table 1: Tanning process**

| **Step n° Operation** | **chemical** | **%** | **Time min** | **T (°C)** | **pH** | **Comments** |
|---|---|---|---|---|---|---|
| | Water | 150 | | 20 | | |
| | Oxalic acid | 0.5 | 20 | | | |
| Drain and wash | | | | | | |
| | Water | 70 | | 20 | | |
| | Paralene PGS | 2 | | | | |
| | Sellasol SL | 2 | 30 | | | |

| **tannage** | | | | | | |
|---|---|---|---|---|---|---|
| | Quebracho ATO | 10 | | | | |
| | Mimosa | 5 | | | | |
| | Chestnut Bark | 5 | 60 | 20 | | |
| Drain | | | | | | |

| **Retan** | | | | | | |
|---|---|---|---|---|---|---|
| | Water | 100 | | | | |
| | Apple Extract | 45 | | | | |
| | Chestnut Bark | 5 | | | | |
| | Fitapor GT | 5 | | | | |
| | Manacryl SRG | 1.5 | | | | |
| | Dermadol ID | 1 | 6 hours + 5 min/hour | 30 | | Run automatically overnight |
| Drain | | | | | | |
| | | | | | | |
| | Water | 100 | | 30 | | |
| | Oxalic acid | 0.50 | | | | |
| Drain and wash | | | | | | |

| **Neutralise** | | | | | | |
|---|---|---|---|---|---|---|
| | Water | 50 | | 40 | | |
| | Sodium formate | 2 | | | | |
| | Dermaflex FR/C | 4 | 15 | | | pH 4.5 - 4.8 |

| **Fatliquor** | | | | | | |
|---|---|---|---|---|---|---|
| | Dermadol BK | 8 | | | | |
| | Dermadol MC | 4 | | | | |
| | Dermadol ID | 2 | | | | |
| | Tresin MG Liq | 5 | 60 | | | |
| | | | | | | |
| | Oxalic acid | 0.3 | | | | |

| **Retan** | | | | | | |
|---|---|---|---|---|---|---|
| | Remsol ALM | 1 | 15 | | | |

| **Fixation** | | | | | | |
|---|---|---|---|---|---|---|
| | Formic acid | 1 | 20 | | | |

## Claims

1. A method of tanning hides or skins, the method comprising,
a fruit tanning step of contacting, for a predetermined time and at a predetermined temperature, a hide or skin with a tanning liquor comprising a fruit tanning extract, **characterised in that** the fruit tanning extract is derived from cider apples, and wherein the tanning liquor also comprises one or more vegetable or synthetic tanning agents, and **in that** the fruit tanning step is a fruit re-tannage step, the predetermined time is from 6 to 48 hours and the predetermined temperature is from 25°C to 85°C.

2. A method as claimed in claim 1, further comprising one or more further tannage steps.

3. A method as claimed in either claim 1 or claim 2, further comprising one or more of the following steps after the fruit tanning step: neutralisation, fatliquoring, fixation and finishing.

4. A method as claimed in any one of the preceding claims, further comprising one or more of the following steps before the fruit tanning step: soaking, liming and/or dehairing, fleshing, splitting, pickling, samming and shaving.

5. A method as claimed in any one of the preceding claims, further comprising one or more tannage steps before the fruit re-tannage step.

6. A method as claimed in any one of the preceding claims, wherein the predetermined time is from 6 hours to 36 hours.

7. A method as claimed in any one of the preceding claims, wherein the predetermined time is from 12 hours to 24 hours.

8. A method as claimed in any one of the preceding claims, wherein the predetermined temperature is from 25°C to 50°C.

9. A method as claimed in any one of the preceding claims, wherein the predetermined temperature is from 25°C to 40°C.

10. A method as claimed in any one of the preceding claims, wherein the fruit tanning extract in obtainable by aqueous extraction of pulped fruit at elevated temperature.

## Patentansprüche

1. Verfahren zum Gerben von Fellen und Häuten, wobei das Verfahren Folgendes beinhaltet:
einen Obstgerbschritt, um für eine vorbestimmte Zeit und bei einer vorbestimmten Temperatur ein Fell oder eine Haut mit einer einen Obstgerbextrakt enthaltenden Gerbbrühe in Kontakt zu bringen, **dadurch gekennzeichnet, dass** der Obstgerbextrakt von Mostäpfeln gewonnen wird und wobei die Gerbbrühe auch ein oder mehrere pflanzliche oder synthetische Gerbmittel enthält, und dadurch, dass der Obstgerbschritt ein Obstnachgerbschritt ist, wobei die vorbestimmte Zeit 6 bis 48 Stunden und die vorbestimmte Temperatur 25°C bis 85°C beträgt.

2. Verfahren nach Anspruch 1, das ferner ein oder mehrere Gerbschritte beinhaltet.

3. Verfahren nach Anspruch 1 oder Anspruch 2, das ferner einen oder mehrere der folgenden Schritte nach dem Obstgerbschritt beinhaltet: Neutralisierung, Fettung, Fixierung und Veredelung.

4. Verfahren nach einem der vorherigen Ansprüche, das ferner einen oder mehrere der folgenden Schritte vor dem Obstgerbschritt beinhaltet: Einweichen, Kalken und/oder Enthaaren, Entfleischen, Teilen, Beizen, Abwelken und Falzen.

5. Verfahren nach einem der vorherigen Ansprüche, das ferner einen oder mehrere Gerbschritte vor dem Obstnachgerbschritt beinhaltet.

6. Verfahren nach einem der vorherigen Ansprüche, wobei die vorbestimmte Zeit 6 Stunden bis 36 Stunden beträgt.

7. Verfahren nach einem der vorherigen Ansprüche, wobei die vorbestimmte Zeit 12 Stunden bis 24 Stunden beträgt.

8. Verfahren nach einem der vorherigen Ansprüche, wobei die vorbestimmte Temperatur 25°C bis 50°C beträgt.

9. Verfahren nach einem der vorherigen Ansprüche, wobei die vorbestimmte Temperatur 25°C bis 40°C beträgt.

10. Verfahren nach einem der vorherigen Ansprüche, wobei der Obstgerbextrakt durch wässrige Extraktion von Fruchtfleisch bei erhöhter Temperatur erhalten werden kann.

## Revendications

1. Procédé de tannage de cuirs et de peaux, le procédé comprenant,
une étape de tannage aux fruits consistant à mettre en contact, pour une durée prédéterminée et à une température prédéterminée, un cuir ou une peau avec une liqueur de tannage comprenant un extrait tannant aux fruits, **caractérisé en ce que** l'extrait tannant aux fruits est dérivé de pommes à cidre, et dans lequel la liqueur de tannage comprend également un ou plusieurs agents tannants aux légumes ou synthétiques, et **en ce que** l'étape de tannage aux fruits est une étape de re-tannage aux fruits, la durée prédéterminée est de 6 à 48 heures et la température prédéterminée est de 25° C à 85° C.

2. Procédé selon la revendication 1, comprenant en outre une ou plusieurs étapes de tannage supplémentaires.

3. Procédé tel que revendiqué soit à la revendication 1, soit à la revendication 2, comprenant en outre une ou plusieurs des étapes suivantes après l'étape de tannage aux fruits : neutralisation, corroyage, fixation et finition.

4. Procédé tel que revendiqué dans l'une quelconque des revendications précédentes, comprenant en outre une ou plusieurs des étapes suivantes avant l'étape de tannage aux fruits : trempe, pélanage et/ou épilage, écharnage, refendage, piclage, essorage et dérayage.

5. Procédé tel que revendiqué dans l'une quelconque des revendications précédentes, comprenant en outre une ou plusieurs étapes de tannage avant l'étape de re-tannage aux fruits.

6. Procédé tel que revendiqué dans l'une quelconque des revendications précédentes, dans lequel la durée prédéterminée est de 6 heures à 36 heures.

7. Procédé tel que revendiqué dans l'une quelconque des revendications précédentes, dans lequel la durée prédéterminée est de 12 heures à 24 heures.

8. Procédé tel que revendiqué dans l'une quelconque des revendications précédentes, dans lequel la température prédéterminée est de 25° C à 50° C.

9. Procédé tel que revendiqué dans l'une quelconque des revendications précédentes, dans lequel la température prédéterminée est de 25° C à 40° C.

10. Procédé tel que revendiqué dans l'une quelconque des revendications précédentes, dans lequel l'extrait tannant aux fruits peut être obtenu par une extraction aqueuse de fruit pulpé à une température élevée.
